

## UNITED STATES PATENT OFFICE.

AUGUSTE ESCAICH AND JEAN PAUL WORMS, OF PARIS, FRANCE.

## DYEING PROCESS.

No Drawing. Application filed November 20, 1923, Serial No. 675,961, and in Germany November 25, 1922.

A dyeing process utilizing nitrous acid in the presence of metallic salts has already been proposed, but practice has shown that this process was not practical, because the bath must be strongly heated and for a long time with the products to be dyed and in the presence of a large quantity of mineral acids—because only brown colors are produced, and because the treated fibres are thus seriously deteriorated or destroyed; this process is unusable for the treatment of leathers and furs.

The present invention has for its object a dyeing process utilizing nascent nitrous acid in the presence of metallic compounds which are soluble or rendered soluble, this process being applicable to all animal fibres, leathers and furs at ambient temperature as in the hot state at a temperature below the boiling point.

In this process, the action of nascent nitrous acid resulting from the decomposition of different bodies containing nitrogen, for example and in the most cases, of nitrite in the presence of any kind of acid capable of decomposing the same has for a result to:

1. Produce autogenous colors on fibres.
2. For increasing the available shades:
  - (a) of diazotizable colors developed on fibres in the known conditions at or below the temperature of the melting ice.
  - (b) of basic colorants utilizing the tannins as mordants.

According to the invention:—

1. Animal substances are dyed by hot treatment or by cold treatment in several hours in more or less acid baths containing alkaline nitrites and metallic salts or oxides, both of which latter substances can moreover be incorporated with the fibre as mordants. All the acids capable of liberating the nitrous acid from the nitrites can be employed whether they are mineral or organic, the same applies to the acid-salts (bisulphates, alums, copper sulphate, unsaturated tartrates or citrates etc. etc.), and according as an organic or mineral acid is employed, or according as these acids are mixed together, the specific color, obtained under the action of the metal, may be shaded.

The nitrous acid can also act in the gaseous state, by one of the usual methods of gaseous production (decomposition by water of the

nitrosyl sulphate, reduction of nitric acid by starch or arsenious acid, etc.).

These principles are applicable not only to dyeing proper but also to vapour tinting and printing.

## 1st Example.

20 litres of water  
+ 10 to 40 grms. sodium nitrite  
+ 10 to 40 grms. copper sulphate  
+ soaking about 24 hours cold or very quickly by heating, without it being necessary to cause to boil

give from old rose to purple on a kilogram of silk or of wool immersed from the commencement of the treatment.

If to the same bath are added 50 to 200 grms. of acetic acid at 10° Bé. or the equivalent acid, the tints are more pronounced, this first example proving that the metallic salts can act without any adjuvant.

In the above example in which the metallic compound is copper sulphate, the obtained color is rosy or purple. Other metallic substances will dye the fibres in the same conditions in other colors which correspond respectively to the utilized metals, for example the zinc salts give a mahogany coloration either in the cold or hot state, and so on.

In all cases, with regard to the proportions of nitrite or of acid (or the equivalent) it is not necessary to confine oneself to the chemical equation:



In the cold treatment on leathers, it is possible to decrease the quantities of acids.

Also the proportions of metallic salts is not fixed and will vary with the desired tints.

All the metallic salts will give results while using very small amounts (0.50 grm. per litre of bath if necessary) which allows of employing expensive products such as uranium or salts.

In the said specification and claims, the term soluble is taken in a general sense and not in the restricted sense as is often the case when the only considered solvent is water.

The multiplication of the tints is in relations with that of the metallic salts. If each of these does not develop a colour in itself, it must nevertheless be remembered that variable yellows be derived from alkaline alums, from corrosive sublimate from molybdates, tungstates, manganese salts, potassium ferricyanide, and the like; reds from nickel, copper salts etc. and greens from cobalt salts etc.

The whole of the metallic salts is thus avail-

55

70

75

80

85

90

105

able whatever may be the acid generating the salt.

The metallic oxides fixed on fibres as mordants give similar results.

5 The present process can be carried out in different ways either by using different mixtures of fibres or by varying the metallic compounds and their proportion in the dyeing bath; also, when varying the proportions 10 of metallic compounds, it will be possible to vary the shades either by applying the above described process to fibres which have already been dyed by known processes by means of diazo colors which require the use of ice, or 15 by using, in order to decompose the employed nitrite, different acids or their equivalents, whereof the quality and quantity can also be varied.

What we claim is:—

20 1. A process for dyeing on animal fibres, consisting in causing to act upon the said fibres at a temperature ranging from the ordi-

nary air temperature to the boiling point of water, of a soluble metallic compound in the presence of nascent nitrous acid.

25 2. A process for dyeing on animal fibres, consisting in causing the action upon the said fibres at a temperature comprised between the ordinary air temperature and the boiling point of water, a soluble metallic compound 30 in the presence of an alkali metal nitrite and of any acid by which nascent nitrous acid is produced in the bath.

3. A process for dyeing on animal fibres, consisting in mordanting said fibres with a 35 soluble metallic compound and in causing to act nascent nitrous acid upon said mordanted fibres, at a temperature ranging from the ordinary air temperature to the boiling point of water.

In testimony that we claim the foregoing as our invention we have signed our names.

AUGUSTE ESCAICH.  
JEAN PAUL WORMS.